

March 22, 1960

L. W. SPROULE ET AL

2,929,782

PHYSICAL COMBINATION OF CALCIUM AND LITHIUM  
HYDROXY STEARATES FOR FORMING GREASES

Filed July 17, 1957



Lorne W. Sproule  
Warren C. Pattenden Inventors

By *L. a. Steinbeck* Attorney

1

2,929,782

**PHYSICAL COMBINATION OF CALCIUM AND LITHIUM HYDROXY STEARATES FOR FORMING GREASES**

Lorne W. Sproule, Sarnia, Lambton, Ontario, and Warren C. Pattenden, Courttright, Lambton, Ontario, Canada, assignors to Esso Research and Engineering Company, a corporation of Delaware

Application July 17, 1957, Serial No. 672,432

3 Claims. (Cl. 252—40)

The present invention is concerned with improved lubricating greases based on the use of a thickening amount of a novel "physical combination" of calcium and lithium 12-hydroxy stearates.

This application is a continuation-in-part of Serial No. 316,302, "Calcium-Lithium Hydroxy Fatty Acid Soap Greases," filed October 22, 1952, by the present inventors and now abandoned.

In brief compass, this invention proposes a lubricating grease composition comprising a lubricating oil thickened with a grease thickener formed at a temperature in the range of 275° to 315° F. by saponification of 12-hydroxy stearic acid with a base comprising about 20% lithium hydroxide and 80% calcium hydroxide, so that the calcium and lithium soaps are simultaneously formed in a proper ratio to obtain a novel physical combination of the two soaps having properties unexpectedly different from the known properties of the individual soaps. This new physical combination of the soaps is an excellent grease thickener in itself, but it can also be combined with other conventional grease thickening soaps, especially with additional amounts of lithium 12-hydroxy stearate.

As the art of grease manufacturing has become more sophisticated, it has been realized that greases having greatly improved properties over the simple soap greases could be prepared by judicious combinations of different basic materials, different soaps of perhaps different chain lengths, configuration and substituent groups, and/or salts, either inorganic salts or salts of low molecular weight carboxylic acids. Quite often it has been found that such combinations of materials unexpectedly result in new types of thickeners, usually broadly termed "complexes," which account for the improved properties of the grease products. These "complexes" often have properties, such as X-ray diffraction patterns, inconsistent with a mere physical blend of the components and can be of many types. It is believed, for example, that the complex formed between a C<sub>12</sub> or higher carboxylic acid soap and calcium acetate at a temperature above 425° F. is of the ionic type, and results in a new crystalline soap structure. "Chemical complexes" of various natures are believed to be formed between low molecular weight dicarboxylic acid salts and soaps.

The art of grease manufacture has not evolved to a point where these complexes are so well known that the "tailor making" of a product involves the simple selection of known ingredients. Extensive experimentation and development are still called for, and quite often unexpected results are obtained.

Mixed calcium and lithium stearate greases have been known to the art. In order to make a satisfactory grease, the lithium component must be present in the thickener in an amount in excess of about 50 wt. percent, which makes the grease excessively expensive. These greases also are deficient in their mechanical stability and oxidation resistance.

Lithium 12-hydroxy stearate greases have also been known to the art, but are also excessively expensive.

2

These greases are valued for their high dropping points. Their water resistance leaves something to be desired, the conventional calcium greases usually giving better service in the presence of water. In order to use a minimum amount of thickener in a grease, the lithium soaps must be prepared at a temperature above 400° F.

Ca 12-hydroxy stearate greases have also been disclosed in the art, and are valued because they do not have to be plasticized with water. Their dropping points, however, do not exceed 290° F., and they must be prepared at relatively low temperatures in the order of 275° F. It has also been found, and this is believed to be unappreciative by the art, that calcium 12-hydroxy stearate greases are very water sensitive. They will break down and fluidize in the presence of more than 0.4 wt. percent water when worked at temperatures above about 190° F. This is objectionable, for example, in equipment such as food can closing units wherein the grease must lubricate at 200° F. in the presence of condensed steam.

From this knowledge of the art, it is believed that in the present invention, it is unexpected that a superior grease thickener comprising lithium and calcium soaps in a novel physical combination could be prepared at a relatively low temperature using only 20 wt. percent lithium through the use of 12-hydroxy stearic acid in place of the unsubstituted acids. It has also been found that this novel physical combination permits a lesser amount of total soap to be used in forming the grease. This use of such a minor amount of lithium in the thickener, the use of less thickener, and the lower manufacturing temperature, are very important from an economic standpoint, as will be appreciated by those skilled in the art.

One unexpected feature of this invention is that the water sensitivity of the calcium 12-hydroxy stearate grease is completely overcome by modifying it by physically combining it with a minor amount of the lithium soap. It would have been expected that the lithium soap would not improve the water sensitivity of the calcium soap, because the latter is generally considered to be superior in water resistance. For example, lithium oleate will practically dissolve in water, while calcium oleate will not.

Another unexpected feature of this invention is that this novel physical combination can be prepared at moderate temperatures in the range of 275°-315° F. This is above the maximum temperature permissible in the manufacture of the calcium soaps, and well below the high temperatures, 400° F. +, necessary to form the lithium soaps. It would have been expected that, at this lower temperature, the lithium soap molecules would not have been sufficiently mobile to enter into a physical combination.

It must be appreciated that this new physical combination of the soaps cannot be arrived at by simple blending of the individual soaps, whether or not this is followed by heating. An unsatisfactory product is obtained by simply blending the components. The two soaps must be simultaneously formed by a co-saponification of the 12-hydroxy stearic acid at a temperature in the range of 275°-315° F. in order to achieve the desired physical combination. The two saponifying agents can be added simultaneously to the acid solution, or one can be added after the other, so long as the saponification because of the first added agent is not substantially complete. The two saponifying agents are preferably blended in plant scale operations with the acid solution within 10 minutes of each other.

The formation of the novel physical combination of soaps of this invention occurs uniquely at about a 20% lithium soap content, although to permit a little latitude

this is given as being in the range of 18 to 22% in the attached claims. Greater amounts of lithium soap do not cause the formation of further amounts of the physical combination and the thickener partakes of the properties of a blend between the 20% lithium/80% calcium physical combination, and the remaining lithium soap that is present. If a lesser amount of lithium soap is used, say 15 wt. percent, the calcium 12-hydroxy stearate is not modified sufficiently to overcome the above described water sensitivity.

This invention will become clear from the following examples and description with reference to the drawing attached to and forming a part of this specification.

The drawing is a graphical presentation of the relationship between the calcium and lithium ratio of the soap and the worked penetration of the grease product, at a total soap content of 10 wt. percent. This graph demonstrates the formation of the novel physical combination of soaps of this invention.

Greases in accordance with the present invention can be prepared as follows: 12-hydroxy stearic acid or an equivalent material is charged to a grease kettle and heated therein to about 180°-200° F., preferably in the presence of an equal weight of lubricating oil, while stirring. The lime is then added, preferably in the form of a water slurry while heating and mixing are continued. After about 3-10 minutes, the lithium hydroxide is added, usually as an aqueous solution. The mixture is then further heated at about 275° to 315° F., preferably 300°-310° F., until dehydration is complete, which can require about 3-6 hours. If desired, further lubricating oil is added as the grease thickens in the course of the dehydration process.

After dehydration is complete, the kettle contents are cooled while stirring. Oil is added while cooling progresses until the desired soap content is reached. It has been found that this soap content need not exceed 15 wt. percent and is usually below 10 wt. percent for a grease based on the novel physical combination of soaps alone.

After oiling the grease back, the grease can be finished by working or milling, as in a Manton-Gaulin homogenizer or Morehouse mill. After or during milling, further oil can be added, if desired, to bring the worked penetration up to the final desired value.

As mentioned before, the new physical combination of the calcium and lithium 12-hydroxy stearates can be used in combinations with other conventional grease thickeners. These can be simply blended with the novel grease thickener of this invention, followed by heating if desired. It is especially preferred to blend the combination soaps of this invention with additional amounts, in the range of 15 to 25 wt. percent, of lithium 12-hydroxy stearate to obtain a grease especially suitable for the lubrication of railroad car wheel roller bearings. This additional amount of lithium soap in the blend can conveniently be provided by using an excess of the lithium saponifying agent during the co-saponification step, or by blending the physical combination of soaps of this invention with additional lithium soap.

#### EXAMPLE 1

A grease containing less than 12 wt. percent of mixed lithium-calcium 12-hydroxy stearate soap thickener having a lithium to calcium soap ratio of 20:80 was prepared as follows:

A grease mixer was charged with 216 pounds of 12-hydroxy stearic acid and 540 pounds of mineral oil. The paddles were turned on and the mixture was heated. The fatty acids melted in the oil at 180° F. At this point, the lime (25 1/4 pounds) was added in the form of a slurry in 90 pounds of water. About 5 minutes later the lithium hydroxide (7 1/4 pounds) in aqueous solution was added. The flow of steam to the grease kettle jacket was increased and the temperature of the kettle contents was raised to 300° F. At this point, a sample of the grease

was checked for free alkali and found to be 0.2%. This was considered satisfactory. After heating at 290°-300° F. for about 5 hours, the steam was turned off and the kettle contents allowed to cool. A test on the grease for water content at this stage was negative. While cooling from 300° F. to about 200° F., 1181 pounds of mineral oil were slowly added, along with 10 pounds of phenyl-alpha-naphthylamine dissolved in 10 pounds of oil. The finished grease was drawn from the mixer into containers at 190° F. This grease required no milling. The composition and properties of the grease are summarized in Table I.

Table I

|    |                               |       |
|----|-------------------------------|-------|
| 15 | Formula, percent by weight:   |       |
|    | 12-hydroxy stearic acid       | 10.8  |
|    | Lithium hydroxide monohydrate | 0.36  |
|    | Hydrated lime                 | 1.26  |
| 20 | Mineral oil <sup>1</sup>      | 87.08 |
|    | Phenyl-alpha-naphthylamine    | 0.5   |

#### Inspections:

|    |                                                 |             |
|----|-------------------------------------------------|-------------|
| 25 | Percent soap:                                   |             |
|    | As Li 12-hydroxy stearate                       | 2.3         |
|    | As Ca 12-hydroxy stearate                       | 9.3         |
| 30 | Free acid, percent oleic                        | 0.28        |
|    | Excess alkali, percent LiOH.H <sub>2</sub> O    | 0.1         |
|    | Worked penetration, 77° F.                      | 275         |
|    | Mechanical stability, penetration after 10,000  |             |
|    | strokes in fine hole worker                     | 295/105° F. |
|    | Water absorption (mixer method) at 150°         |             |
| 35 | F.: No. of ccs. of water absorbed               | 11          |
|    | (Consistency good)                              |             |
|    | ASTM dropping point, ° F.                       | 318         |
|    | Wheel bearing test, 6 hrs. at 220° F. and       |             |
|    | 60 m.p.h.:                                      |             |
|    | Gms. of grease leakage                          | 1.4         |
| 40 | Over-all rating                                 | Good        |
|    | Spindle test, hrs. at 250° F. and 10,000 r.p.m. | 1100        |
|    | App. viscosity at 100 spec. <sup>-1</sup> :     |             |

#### Shear (Strokes):

|    |         |     |
|----|---------|-----|
| 45 | 77° F.  | 180 |
|    | 130° F. | 68  |
|    | 175° F. | 38  |
|    | 200° F. | 30  |
| 50 | 225° F. | 23  |
|    | 250° F. | 24  |
|    | 275° F. | 27  |
|    | 300° F. | 9.5 |

#### Bleeding—percent oil loss after 100 hrs. at 225°

|    |    |   |
|----|----|---|
| 55 | F. | 6 |
|----|----|---|

<sup>1</sup> Viscosity 60 SUS at 210° F., and a viscosity index of 50.

It will be noted that this grease, in spite of its low total soap content and very low lithium soap content, has a satisfactory dropping point above 300° F., excellent working properties, very high water resistance and excellent bearing performance.

#### EXAMPLE 2

Four additional greases were prepared besides grease "A" of Example 1. The three lithium containing greases, B, C, and D were prepared in a manner similar to that of Example 1 at a saponification and dehydration temperature of about 300°-310° F. Grease E, a 100% calcium grease, was prepared by melting the acid in four times its weight of mineral oil at 180° F. A water slurry of the lime was added in slight excess, and the mixture was then stirred and dehydrated at about 270° F., the maximum permissible temperature. This required about 14 hours. When dehydration was complete, further oil was added to adjust the soap content. The oil used for these greases

was the same as in Example 1. Table II gives the inspections and tests of these greases.

Table II

| Grease                                                                                               | B    | C    | D    | A         | E     | 5  |
|------------------------------------------------------------------------------------------------------|------|------|------|-----------|-------|----|
| Percent Lithium Soap in thickener                                                                    |      |      |      |           |       |    |
| Percent soap after oiling back end milling                                                           | 100  | 40   | 20   | 20        | 0     |    |
| Worked penetration at 77° F.                                                                         | 15.3 | 14.3 | 12.5 | 11.6      | 15    | 10 |
| ASTM Dropping Point, ° F.                                                                            | 328  | 280  | 280  | 275       | ----- |    |
| ASTM Micro-penetration at 77° F. of grease containing 5 wt. percent water, mixed at room temperature | 331  | 318  | 318  | 318       | ----- |    |
| ASTM Micro-penetration at 77° F. after heating at 200° F. under 50 lbs./sq. in. nitrogen pressure:   |      |      |      | 80        | 38    |    |
| After 3 hours                                                                                        |      |      |      | No change | Fluid |    |
| After 6 hours                                                                                        |      |      |      | 68        | ----- |    |

The data of Table II show the effect of substituting

ing properties. When the calcium 12-hydroxy stearate is modified, however, in accordance with this invention, the properties of the new crystalline structure are such as to yield fibers having good properties.

## EXAMPLE 3

Nine additional greases were prepared having a total soap content of 10 wt. percent, in a base oil similar to that of Example 1. Products F and G, consisting mostly of the calcium soap, were of necessity prepared at a somewhat lower temperature. Table III gives the results and inspections of the grease products F through N. The attached drawing graphically illustrates by the dashed line the relationship between the lithium-calcium ratio of the greases, and the worked penetration of these grease products. The solid line on the graph illustrates the worked penetration of greases having comparable lithium-calcium ratios, but prepared by simple blending of the two soaps rather than by co-saponification.

Table III

|                                                                                                                      | F(1) | G(1) | H   | I   | J     | K     | L     | M     | N     |
|----------------------------------------------------------------------------------------------------------------------|------|------|-----|-----|-------|-------|-------|-------|-------|
| Percent of Soap which is lithium(2)                                                                                  | 0    | 5    | 12  | 20  | 23    | 40    | 60    | 80    | 100   |
| Worked Penetration                                                                                                   | 280  | 284  | 274 | 279 | 281   | 318   | 336   | 378   | 400   |
| Dropping Point                                                                                                       | 290  | 292  | 288 | 318 | 320   | 327   | 342   | 364   | 378   |
| Percent Change in Penetration after 16 hours at 200° F. under 50 lbs. nitrogen pressure (grease mixed with 5% water) | 168  | 128  | 71  | 0   | ----- | ----- | ----- | ----- | ----- |

<sup>1</sup> F prepared at 265° F.; G prepared at 280° F.; all other products made at 300°-310° F.

<sup>2</sup> Balance is calcium.

a minor portion of lithium for the calcium in the hydroxy stearate greases. Grease B requires substantially more than 15.3% soap in order to obtain a grease having a worked penetration of about 280. The amount of soap necessary would be less if grease B had been prepared at a higher temperature of about 400° F. Greases A and D illustrate the novel physical combination of soaps of this invention, and show that only 12.5 wt. percent or less soap is needed to achieve the desired penetration. Grease C illustrates this physical combination of soaps with an additional 20% thickener comprising of lithium 12-hydroxy stearate.

For comparison, a grease prepared with stearic acid, rather than the hydroxy acid, having a lithium-calcium ratio of 40/60 and a total soap content of 15 wt. percent, has a worked penetration of 395. Stearic acid is, therefore, not a suitable ingredient in this type of grease prepared at 275°-315° F.

The last two inspections of Table II give the results of testing the water sensitivity of the greases. Grease A was substantially unaffected by the water, while the 100% calcium grease rapidly fluidized.

A calcium 12-hydroxy stearic grease hardens as the water content decreases during the dehydration step. Thus, a calcium 12-hydroxy stearic grease containing 20 wt. percent soap and 0.5 wt. percent water, while being dehydrated at 260° F., is semi-fluid. When the water content is reduced to 0.05%, the work penetration is 142. The effect of the water in the calcium 12-hydroxy stearic grease is reversible about 190—200° F. For example, if water is mixed with a calcium 12-hydroxy stearic grease at 200° F., it reverts to a fluid product. When, however, 20% of the total soap of the grease is formed from lithium 12-hydroxy stearate by co-saponification in the manner of this invention, the grease product does not become fluid when heated in the presence of water above 200° F. While the reason for this is not certain, it is believed that above 200° F. calcium 12-hydroxy stearate exists as a monohydrate. The geometry of this monohydrate crystal is probably such as to form poor fibers having inferior grease thickening.

35 Table III and the drawing clearly illustrate that there is a new type of structure, or new physical combination, formed by the lithium and calcium 12-hydroxy stearic soaps when they are in the ratio of 20% lithium and 80% calcium, and when they are prepared by co-saponification.

40 The graph shows the sharp change in the worked penetration of the grease products that occurs when the lithium content reaches about 20%. This is indicative of the formation of the novel physical combination of soaps of this invention.

45 Examples 2 and 3 together show the remarkable water insensitivity imparted to the calcium 12-hydroxy stearate by properly physically combining it with about 20% of the lithium soap, and also clearly show that the full benefits of this invention are not obtained by using less than about 20% of the lithium soap.

## EXAMPLE 4

55 To demonstrate that the physical combination of the soaps can be attained only by co-saponification, the following tests were carried out: The 100% calcium grease, grease F of Table II, was blended with the 100% lithium grease, grease B, to obtain two greases, each having a soap content of 10 wt. percent, and a lithium/calcium ratio of 20/80. One grease, grease L, was blended at 75° F.; and the other, grease M, at 200° F. These greases were tested with the following results:

Table IV

| Grease                                                                           | L   | M   |
|----------------------------------------------------------------------------------|-----|-----|
| Worked penetration at 77° F.                                                     | 290 | 295 |
| Dropping Point, ° F.                                                             | 288 | 288 |
| ASTM Micro-penetration at 77° F. of grease containing 5% water, percent increase | 17  | 16  |

70 The attached drawing illustrates the results obtained by blending different amounts of the soaps to obtain several more greases. Comparison of the two lines shows

that a product having different physical properties is prepared by cosaponification.

This example shows that the novel physical combination of soaps, according to this invention, cannot be obtained by simple blending of the components, but that it must be formed by co-saponification at 275°-315° F.

#### EXAMPLE 5

When the amount of lithium saponifying agent used is in excess of the "natural" ratio of 20%, the excess lithium soap is simply blended with physical combination of soaps. This is illustrated by the following: Two greases were prepared at 300° F., similar to greases F and N of Table III, each having a total soap content of 10 wt. percent. These two greases, one having 100% lithium soap and the other 20% lithium and 80% calcium soaps, were then blended at about 100° F. to achieve a grease wherein the thickener comprised 40% lithium soap and 60% calcium soaps. This blend contained 10 wt. percent of total soap and had a dropping point of 332° F. and a worked penetration at 77° F. of 293. It can then be seen that this "blend" had properties substantially equivalent or slightly superior to the cosaponified greases, grease C of Table II and grease K of Table III.

This example shows that grease products containing the new physical combination of soaps of this invention, but containing more than 20% lithium, can be prepared by either cosaponification of the acid using a base containing the desired ratio of lithium to calcium, or by blending the desired additional amount of lithium soap with the physical combination of soaps after it has been formed by co-saponification.

#### EXAMPLE 6

The greases of the present invention can be combined with other conventional additives such as thickeners, antioxidants, corrosion inhibitors, tackiness agents, load-carrying compounds, viscosity index improvers, oiliness agents, etc. These additives can be incorporated at any suitable stage of the manufacturing process as will be understood by those skilled in the art. A grease containing additives was prepared for the purpose of steel mill lubrication from the following ingredients:

|                                              | Pounds |
|----------------------------------------------|--------|
| 12-hydroxy stearic acid                      | 237    |
| Mineral oil charged to mixer with fatty acid | 360    |
| Lime                                         | 28     |
| Lithium hydroxide                            | 8      |
| Balance of mineral oil                       | 2089   |

At 170° F., the following materials were added to impart extreme pressure characteristics to the grease:

|                                                     | Pounds |
|-----------------------------------------------------|--------|
| Chlorinated paraffin wax containing 40% chlorine    | 60     |
| Sulfurized sperm oil                                | 180    |
| Lead naphthenate (containing about 30% lead as PbO) | 37.5   |

The mineral oil used was a mixture of two low cold test mineral oil distillates blended to give a viscosity at 210° F. of 110 SUS. One oil in the blend had a viscosity at 210° F. of 170/190 SUS, while the other oil had a viscosity at 210° F. of 53/57 SUS. The composition and characteristics of this grease are summarized below.

Composition, percent by weight:

|                          |       |
|--------------------------|-------|
| 12-hydroxy stearic acid  | 7.90  |
| Lithium hydroxide        | 0.27  |
| Hydrated lime            | 0.94  |
| Distillate 170/190       | 57.00 |
| Distillate 53/57         | 24.64 |
| Chlorinated wax (40% Cl) | 2.00  |
| Lead naphthenate         | 1.25  |
| Sulfurized sperm oil     | 6.00  |

#### Inspections:

|                                                                   |     |
|-------------------------------------------------------------------|-----|
| Mineral oil viscosity at 210° F., SUS                             | 110 |
| Worked penetration                                                | 305 |
| Dropping point, ° F.                                              | 312 |
| Timken O.K. load (lbs.)                                           | 43  |
| Bleeding test <sup>1</sup> : percent oil loss—100 hrs. at 225° F. | 3.9 |
| Water wash test at 150° F. <sup>2</sup> : percent grease loss     | 12  |

<sup>1</sup> 185 grams of grease in a 28 mesh galvanized cone.

<sup>2</sup> AN-G. 15 specification.

Conventional animal, vegetable, mineral or synthetic oils can be used to form the grease compositions of this invention. Examples of the latter are di-2-ethyl hexyl sebacate, silicone oils, phosphonates, and complex synthetic esters formed from alcohols, dicarboxylic acids and glycols. Preferably the oils used have a viscosity in the range of 10 to 200 SSU at 210° F. and a viscosity index in the range of 30 to 140. It is preferred to use 12-hydroxy stearic acid as an initial ingredient, but equivalent materials that yield the acid under the saponification conditions can also be used. For example, esters of the acid that yield alcohols boiling above 315° F. can be used as a source of the acid. The total soap content of the greases of this invention can range from 5 to 15 wt. percent, and the physical combination of soaps can comprise from 75 to 100% of the grease thickener. The preferred grease compositions of this invention have a dropping point above 320° F. and a worked penetration in the range of 300 to 360.

Having described this invention, what is sought to be protected by Letters Patent is succinctly set forth in the following claims.

What is claimed is:

1. A lubricating grease comprising a major amount of mineral lubricating oil and a grease thickening amount of a mixed-metal thickener prepared by co-saponifying in said lubricating oil 12-hydroxy stearic acid with lithium base and calcium base, heating to a temperature of 275° to 315° F. to dehydrate, and cooling to form said grease, wherein the proportion of lithium to calcium base is such that said mixed-metal thickener consists of 18 to 22 wt. percent lithium 12-hydroxy stearate and 82 to 78 wt. percent of calcium 12-hydroxy stearate.

2. A lubricating grease comprising a major amount of mineral lubricating oil and a grease thickening amount of a soap thickener to form a final grease wherein 15 to 25% of the total soap present is lithium 12-hydroxy stearate and the remainder of said soap is mixed lithium-calcium 12-hydroxy stearate which is prepared by co-saponifying in a mineral lubricating oil 12-hydroxy stearic acid with lithium and calcium hydroxide, heating to a temperature of 275° to 315° F. to dehydrate to thereby form a mixed calcium-lithium 12-hydroxy stearate grease, the proportion of lithium hydroxide to calcium hydroxide being such that said mixed calcium-lithium 12-hydroxy stearate consists of 18 to 22 wt. percent lithium 12-hydroxy stearate and 82 to 78 wt. percent of calcium 12-hydroxy stearate, mixing with said calcium-lithium 12-hydroxy stearate grease a second grease comprising mineral lubricating oil thickened to a grease consistency with lithium 12-hydroxy stearate.

3. A lubricating grease prepared by co-saponifying in mineral lubricating oil 12-hydroxy stearic acid with a lithium base and calcium base, heating to a temperature within the range of 275° to 315° F. to dehydrate, and cooling to form said grease, wherein said lubricating oil has a viscosity of 10 to 200 SSU at 210° F. and a viscosity index of 30 to 140, wherein the amount of lithium to calcium base is such as to result in a thickener consisting of 20% lithium 12-hydroxy stearate and 80% calcium 12-hydroxy stearate, said lubricating grease having

a dropping point above 320° F. and a work penetration  
at 77° F. of 300 to 360 mm./10.

References Cited in the file of this patent

UNITED STATES PATENTS

2,397,956 Fraser ----- Apr. 9, 1946  
2,542,159 Stevens ----- Feb. 20, 1951

2,607,735 Sproule et al. ----- Aug. 19, 1952

OTHER REFERENCES

5 The Manufacture and Application of Lubricating  
Greases, Boner, Reinhold Pub. Corp., New York, 1954,  
pp. 599 and 600.